# EUROPEAN PATENT SPECIFICATION

(11) **EP 0 160 761 B1**
(45) Date of publication and mention of the grant of the patent: **08.02.1989**
(21) Application number: 84303633.6
(22) Date of filing: 30.05.1984
(51) Int. Cl.: C25D 3/56, C25D 5/10, C25D 7/00, H01H 1/02

(54) **Amorphous transition metal alloy, thin gold coated, electrical contact**
Elektrischer Kontakt beschichtet mit einer amorphen Übergangslegierung der selbst mit einem Goldfilm beschichtet ist
Contact électrique revêtu d'un alliage amorphe d'un métal de transition lui-même revêtu d'un film d'or

(30) Priority: 11.05.1984 US 609137
(43) Date of publication of application: 13.11.1985
(73) Proprietor: Burlington Industries, Inc., Greensboro North Carolina 27420 (US)
(72) Inventor: Gamblin, Rodger Lotis, Dayton Ohio, 45419 (US)
(74) Representative: Arthur, Bryan Edward

(56) References cited:
- DE-B- 1 059 738
- GB-A- 1 507 782
- US-A- 4 101 389
- METAL FINISHING ABSTRACTS, volume 22, no. 3, May/June 1980, Teddington, Middlesex (GB) page 187H, & JP - A - 54 110470 (HITACHI)
- METAL FINISHING, volume 82, no. 1, January 1984, pages 59-65, C. RAJAGOPAL et al.: "Electrode-deposition of corrosion resistant amorphous nickel alloys on mild steel"

## Description

### Background and summary of the invention

The invention relates to an electrical contact surface (such as an electrical switch contact) having low contact resistance, relatively low cost, acceptable solderability, and high corrosion resistance. The electrical contact surface, and method of formation thereof, according to the present invention are particularly designed to replace conventional electrical contact surfaces wherein a gold layer of at least about 0.762 pm (about 30 microinches) thickness is applied over a crystalline substrate.

In the electrical connector industry where low voltage and/or current signals must be conducted reliably, and in some situations where intermediate voltage and/or current signals must be conducted, gold is currently used to insure low contact resistance, and thus effective conduction. Usually the gold is applied over a crystalline base metal such as copper, brass, or silver, with or without an intermediate strike of nickel, and the thickness of the gold layer is normally at least about 0.762 11m (about 30 microinches) (e.g. 1.27-2.54 11m (50-100 microinches). At a thickness of 1.27 pm (50 microinches) the cost of the gold layer is on the order of 5 cents/cm^{2.} It is the characteristic of gold-with such a thickness-that it is porous and thus through time the underlying material, or its corrosion products, may migrate to the surface of the gold and unacceptably raise the contact resistance. Additionally, certain organic materials or sulfur compounds can polymerize on a gold surface and cause high contact resistance. Additionally, gold has less than ideal solderability since it dissolves in and embrittles some solder alloys.

From an article on pages 59-65 of Metal Finishing, Volume 82, No. 1. January 1984 by C. Rajagopal et al, a method is known of electrodepositing amorphous nickel alloys comprising nickel and phosphorous and optionally boron, on mild steel in'order to provide better corrosion protection and hardness of the deposit.

According to the present invention an electrical contact surface is provided which overcomes the drawbacks associated with the conventional electrical contact surfaces described above, in that in low and intermediate voltage and/or current signal situations effective conduction can be obtained at less cost and over longer periods of time.

According to the present invention, an electrical contact is provided having a contact resistance soon after production of less than 4 milliohms, comprising an electrically conductive substrate, an amorphous transition metal alloy deposited on said substrate, and an uncovered coating of gold over said amorphous transition metal alloy, said gold coating being between about 0.0254-0.762 ₁₁m (1-30 microinches) thick. The electrically conductive substrate is preferably a metal such as copper, bronze, brass, aluminum, or silver, and the amorphous (as opposed to crystalline) transition metal alloy is preferably electrolytically deposited thereon.

An "amorphous" alloy is one that has a geometric or topological configuration of the atoms forming the alloy that is different from crystalline (i.e. non-crystalline). Typically, metal alloys are crystalline. When X-ray diffraction tests are done on crystalline materials, it can be seen that the materials exhibit sharp peaks for the d-spacings between planes in the ordered crystal structure. The narrowness or width of these peaks relative to thick height gives an indication of the size of the crystals. For amorphous materials, there are no particularly sharp peaks, the amorphous material being characterized by lack of order in the atomic structure. The exact nature of the amorphous structures is not known; however there are a number of theories which attempt to describe the configurations of the atoms in amorphous materials. In this regard attention is directed to an article entitled "Metallic Glasses" by Chaudhari et al, appearing in Scientific American, Volume 242, No. 4, 1980, pages 98-117.

The amorphous transition metal alloy according to the invention preferably is a nickel-phosphorus alloy, such as one having about 15-25 atomic percent phosphorus (preferably about 20 percent), with cobalt, or some other transition metals, utilizable in addition to, or in place of, the nickel. Various materials may be added to the plating bath to enhance the corrosion protection of the electrical contact surface being formed, particularly advantageous materials being hexafluosilicate (SiFₛ-), hexafluotitanate (TiFₛ-) or hexafluozirconate (ZrFₛ-) ions.

After the amorphous nickel alloy has been electrolytically deposited on the substrate, the amorphous nickel alloy is coated with a layer of gold. When the amorphous nickel alloy is coated with a layer of gold of a given thickness, the contactor that results exhibits superior properties compared to conventional contactors wherein the same thickness of gold is coated on a crystalline metal alloy. For instance, a gold thickness of less than 0.762 pm (30 microinches) over the amorphous nickel alloy produces an electrical contact structure according to the invention that is equal to, or superior to, conventional contactors wherein a coating of 1.27―2.54 µm (50-100 microinches) of gold is provided. In fact, it is possible to obtain entirely acceptable contactors even when the gold coating is 0.0254 ₁₁m (one microinch) thick (at this thickness the cost of the gold is only about 0.1 cents/cm²), although a range 0.127-0.381 pm (5-15 microinches) is preferred. The electrical contact surface resulting has stable contact resistance both initially and after exposure to a series of common atmospheric corrodants, and initially (soon after production) when tested pursuant to ASTM B667-80 has a contact resistance less than 4 milliohms.

According to another aspect of the present invention, a method of producing an electrical contact surface is provided, comprising the steps of: a) immersing an electrically conductive substrate in a plating bath including transition metal alloying elements; and b) controlling the bath temperature conditions and current density at the cathode to effect electrolytic deposition of the transition metal alloying elements, in amorphous form, on the substrate; and c) applying a coating of gold having a thickness of between 0.0254-0.762 pm (1-30 microinches) to the electrolytically deposited amorphous transition metal alloy, to produce an electrical contact structure having an uncovered gold surface.

Nickel chloride, cobalt carbonate, and phosphorous acid are preferred bath constituents. A number of bath additives can be provided to influence contact resistance and corrosion protection in a positive way. Typical bath additives include boric acid, hydroxyacetic acid, acetic acid, 0-alanine, succinic acid, surfactants of the alkoxylated linear alcoholic class, SiFₛ- ions, TiFₛ- ions and ZrFₛ- ions. The bath temperature conditions, and the current density at the cathode, are maintained so that effective electrolytic deposition takes place.

It is the primary object of the present invention to provide for the production of electrical contact surfaces that have low, stable contact resistance over extended periods of time even when subjected to corrosive conditions, and at a relatively low cost. This and other objects of the invention will become clear from an inspection of the detailed description of the invention and from the appended claims.

### Detailed description

A deposition of an amorphous transition metal alloy can be provided on a substrate by immersing the substrate (or a portion thereof) in a plating bath. Amorphous transition metal alloys have been found to have better corrosion resistance than crystalline materials, and a thinner coating of gold over an amorphous transition metal alloy produces a contactor having the same, or better, properties than a contactor formed by a thicker coating of gold over a crystalline material. Further, acceptable contacts can be obtained, according to the invention, with only a very thin coating of gold.

Typical transition alloys that are useful electrical contact surfaces (such as electrical switch contacts) according to the invention are nickel and cobalt. Nickel is the preferred transition metal since it has the least cost of the most corrosion resistance, of suitable transition metals. However, generally comparable, and sometimes superior, results can be achieved substituting cobalt, for all or part of the nickel, in the plating bath.

An amorphous deposition of the nickel on the conductive substrate (which preferably comprises a metal such as copper, bronze, brass, aluminum, or silver, or alloys thereof) is formed when phosphorous acid is included in the plating bath, and a relatively high percentage of phosphorus is provided in the alloy that is formed. A phosphorus concentration of at least about 12%, and preferably of about 15-25 atomic percent is desired in order to achieve good corrosion resistance and low contact resistance. Most preferably the amorphous deposited alloy has about 20 atomic percent phosphorus.

The bath temperature conditions, and the current density at the cathode, are controlled in order to maximize the corrosion resistance and minimize the contact resistance. Typically current density is about 538.2 amp/m²⁻26909.8 amp/m² (about 50 amp/ft²⁻2500 amp/ft²), with a range of about 1076.4 amp/m²⁻9687.6 amp/m² (about 100-900 amp/ft²) preferred. Typical temperatures are 70-85°C with 75―80°C preferred. Temperature is not critical, but lower temperature will have a tendency to increase the preference of cobalt for nickel in the plating where both are present in the bath.

Various additives may be provided in the bath in order to positively affect the contact resistance and corrosion resistance. When the bath contains hexafluosilicate ions at a concentration of about 0.1 molar to the solubility limit (with the addition of small amounts of HF to maintain solubility if necessary) the overall corrosion resistance of the amorphous nickel alloy may be enhanced. A generally comparable enhancement of corrosion resistance may also be obtained by substituting TiFₛ- or ZrFₛ- ions for part or all of the SiFs- ions.

In a plating bath containing nickel or cobalt ions and phosphorus acid any suitable anode and cathode materials may be utilized. For instance the anode can either be inert (platinized titanium, platinum, or graphite), or can be of nickel (or like transition metal to be deposited). If TiFₛ-, SiFₛ- or ZrFₐ- ions are included in the bath a nickel or cobalt anode must be used. With an inert anode additions of nickel or cobalt must be made from time to time (preferably in the form of NiC0₃ or CoC0₃) to maintain the nickel content. With the nickel anode the content of nickel ion in the bath tends to rise since each two electrons at the anode cause the dissolution of about one nickel ion, while at the cathode both nickel and phosphorus are being reduced. A nickel and an inert anode can be used together such that each carries only a portion of the current, and thus maintains a balanced bath with regard to nickel. Phosphorous, in the form of phosphorous or hypophosphorous acid, and preferably in the form of phosphorous acid, must be added from time to time-irrespective of the anode construction-to maintain the proper bath balance, although the proportion of phosphorous acid is not critical and the bath balance can be maintained rather easily.

After deposition of the nickel phosphorous alloy, or the like, on a substrate, a coating of gold is applied over the amorphous alloy. Preferably this is accomplished by providing an electrodeposit that is applied for a controlled time at a controlled current density. The thickness of the gold coating is determined by the desired end properties of the contactor produced. Within wide ranges, whatever the thickness of the gold coating on the amorphous alloy, the contactor that results can be expected to have enhanced properties compared to contactors formed by the same thickness of gold coating over a crystalline material. In fact, acceptable electric contacts can be produced even when the thickness of the gold coating is about 0.0254 pm (about 1 microinch). Preferably the gold coating is in the range of 0.127-0.762 pm (5―30 microinches), and more preferably 0.127-0.381 pm (5-15 microinches).

The gold used for the coating preferably is hard gold, athough soft gold is also practical although usually with somewhat less desirable results. The thickness of the amorphous transition metal alloy on the substrate is not particularly critical. It merely need be thick enough to achieve the desired results according to the invention. A preferred thickness is in the range of about 1.27-3.81 um (about 50 microinches-150 microiriches). Ranges of 0.635-25.4 µm (25 microinches-1000 microinches) are practical.

In the typical manufacture of an electrical contact according to the invention (which may be of a wide variety of forms, such as edge card connectors, contact leaf springs, rigid electrical switch contact structures, etc.), desirably, the electrically conductive substrate is formed into the desired final contact shape. It is then immersed in a cleaner, and the deionized water, and then a dilute hydrochloric acid solution. Then it is placed in the Ni-Co-P plating bath and after plating it is rinsed in deionized water. Then the gold plating is provided thereon in any conventional way, such as in a gold plating bath maintained at about 30-35°C with a current density of about 107.6 amp/m² (about 10 amp/ft²). After the gold plating is applied it is again immersed in deionized water.

Alternatively, for many electrical contact shapes (such as edge card connectors), it is possible to plate blanks or coupons first, and only after they have been plated and a gold strike applied are they formed into the desired shape.

The following are examples of the practice of the invention.

### Example 1

A plating bath was formed with the following composition:

An electrically conductive substrate was immersed in the bath, which was maintained at a temperature of about 80°C, and with a current density at the cathode of about 150 ma/cm². When removed from the bath, the substrate had an amorphous nickel-phosphorous alloy thereon. A 0.0254 pm (one (1) microinch) strike of gold was provided on the amorphous alloy. The electrical contact surface that resulted had a contact resistance that was substantially as low as a similar substrate with a 1.27 µm (50 microinch) or greater coating of gold, the contact resistance was stable over time, and as stable in corrosive environments (such as when subjected to the S0₂ test-100 percent relative humidity and 1 percent concentration of sulfur dioxide, room temperature, over forty hours-, and the mixed gas test-the same conditions as the S0₂ test only adding 1 percent nitrogen dioxide and 1 percent chlorine). The electrical contact surface formed was much less expensive than the conventional one, and had better solderability characteristics.

### Example 2

In this example, the bath composition, temperature, and current density characteristics were substantially the same as in Example 1. After the substrate with an amorphous nickel-phosphorous alloy was removed from the bath, an approximately 0.254 µm (10 microinch) strike of gold was provided on the amorphous alloy. The electrical contact surface that resulted had contact resistance, and other properties, equal, or superior to, an electrical contact surface formed utilizing similar materials in crystalline form, and with a 1.27 pm (50 microinch) coating of gold.

### Example 3

The bath composition for this example was as follows:

The bath temperature conditions, current density, and like parameters, were substantially the same as for Example 1, and after deposition of the amorphous nickelphosphorous alloy on the substrate a 0.0254 µm (1 microinch) flash of gold was applied. By testing, the electrical contact surface formed was found to have acceptable contact resistance (i.e. less than 4 milliohms when tested according to ASTM B667-80) and corrosion resistance, although it was not as good as the electrical contact surface produced in Example 1.

### Example 4

The bath composition for this Example was as follows: acid

The bath temperature was maintained at about 75°C, with a current density at the cathode of about 200 ma/cm². An analysis of the plating resulting from immersion of the substrate in this bath showed bulk values (in atomic percent) of 6.8±4% cobalt, 0.6 oxygen, 73.3 percent nickel, and 19.3 percent phosphorus. A 0.0254 µm (1 microinch) strike of gold was provided on the amorphous alloy. The electrical contact surface formed had low contact resistance and high corrosion resistance, and was an excellent substitute for conventional electrical contact surfaces of gold about 1.27 µm (about 50 microinches) thick (or thicker) applied over a crystalline base metal.

### Example 5

A number of platings were produced on electrically conductive substrates to produce platings having about 20% phosphorous, X% cobalt, and 80-X% nickel, utilizing the constituents indicated in the following table:

Plating was accomplished at 75-78°C using a hard anode (e.g. platinum or platinized titanium) and a current density of about 1076.4 amp/m² (about 100 amp/ft²).

The sum of the nickel plus cobalt is one mole/liter in each formulation, and CoCOa is the source of all the cobalt in each of the formulations. Therefore, the Co⁺²/Ni⁺² ratio in the bath is M/1 CoCO₃/(-M/1 CoCO₃). The Co/Ni ratio in the plating is %CO(80-%Co). The relationship between Co⁺²/Ni ⁺² in the bath and Co/Ni in the plate is:

It is evident that the cobalt is being plated preferentially to the nickel and that at low cobalt levels this preference is slightly greater. Operating at lower temperature will make the preference (Co/Ni in plating) greater, as will operating at higher current density. Further, these formulations produce lower than nominal amounts of cobalt when they are new, i.e. for the first 100 amp-minutes/liter the baths will produce only ca. 1/2 to 2/3 the desired cobalt content in the plating.

The plating, formed as actual electrical connectors, having 10% Co were coated with 0.127, 0.254 or 0.381 µm (5, 10 or 15 microinches) of hard gold, or 0.127 pm (5 microinches) soft gold, and subjected to durability cycling utilizing conventional techniques, and exposure in a BCL Class III environment, and utilizing the same material on both the PC boards and the connector openings. The following results were achieved, wherein
R_{c}=the contact resistance and
a=a measure of the deviations of the individual contact values from their average

These results indicate improved performance of the electrical connectors according to the invention compared to a 1.27 µm (50 microinch) plating of hard gold over conventional sulfamate nickel.

## Claims

1. An electrical contact having a contact resistance soon after production of less than 4 milliohms, comprising an electrically conductive substrate, an amorphous transition metal alloy deposited on said substrate, and an uncovered coating of gold over said amorphous transition metal alloy, said gold coating being between about 0.0254-0.762 µm (1-30 microinches) thick.

2. An electrical contact as recited in claim 1 characterized in that said transition metal alloy is a nickel-phosphorus alloy.

3. An electrical contact as recited in claim 2 characterized in that said nickel-phosphorus alloy includes about 15-25 atomic percent phosphorus; and includes about 5-15 atomic percent cobalt.

4. An electrical contact as recited in claim 3 characterized in that said uncovered coating of gold is hard gold between about 0.127-0.381 pm about (5-15 microinches) thick.

5. A method of producing an electrical contact comprising the steps of: a) immersing an electrically conductive substrate in a plating bath including transition metal alloying elements; and b) controlling the bath temperature conditions and current density at the cathode to effect electrolytic deposition of the transition metal alloying elements, in amorphous form, on the substrate; and c) applying a coating of gold having a thickness of between 0.0254―0.762 µm (1-30 microinches) to the electrolytically deposited amorphous transition metal alloy, to produce an electrical contact structure having an uncovered gold surface.

6. A method as recited in claim 5 characterized in that step a) is practised utilizing a plating bath containing phosphorus acid and nickel alone, or nickel and cobalt.

7. A method as recited in claim 5 characterized in that step b) is practised so that the temperature of the bath is between about 70-85°C, and so that the current density at the cathode is between about 1076.4-9687.6 amp/m² (100-900 amp/ft²) and to effect an electrolytic deposition of the amorphous material so that it has a thickness of about 0.635-25.4 µm (25-1000 microinches); and that step a) is practised by including in the plating bath between 0.1 molar to the solubility limit of ions selected from the group consisting of TiFₑ- SiFₛ- and ZrFₛ- ions.

8. A method as recited in claim 7 characterized in that steps a) and b) are practised so that the amorphous alloy deposited on the substrate is a nickel cobalt phosphorus alloy, including about 15-25 atomic percent phosphorus, and at least 5 atomic percent cobalt.

9. A method as recited in claim 5 characterized in that step c) is practised so as to apply a coating of hard gold having a thickness of between 0.127-0.381 µm (5-15 microinches).

## Patentansprüche

1. Elektrischer Kontakt mit einem Kontaktwiderstand unmittelbar nach der Herstellung von weniger als 4 mOhm, mit einem elektrisch leitfähigen Susbtrat, einer auf das Substrat aufgebrachten amorphen Übergangsmetallegierung und einer unbedeckten Beschichtung von Gold über der amorphen Übergangsmetallegierung, wobei die Goldbeschichtung zwischen etwa 0,0254-0,762 pm (1 bis 30 microinches) dick ist.

2. Elektrischer Kontakt nach Anspruch 1, dadurch gekennzeichnet, daß die Übergangsmetallegierung eine Nickel-Phosphorlegierung ist.

3. Elektrischer Kontakt nach Anspruch 2, dadurch gekennzeichnet, daß die Nickel-Phosphorlegierung etwa 15-25 Atomprozent-Phosphor enthält; und etwa 5-15 Atomprozent Kobalt aufweist.

4. Elektrischer Kontakt nach Anspruch 3, dadurch gekennzeichnet, daß die unbedeckte Beschichtung mit Gold Hartgold mit einer Dicke zwischen etwa 0,127-0,381 pm (5-15 microinches) dick ist.

5. Verfahren zum Herstellen eines elektrischen Kontaktes mit den Schritten: a) Eintauchen eines elektrisch leitfähigen Substrats in ein Plattierungsbad mit Übergangsmetall-Legierungselementen; und b) Steuern der Badtemperaturbedingungen und der Stromdichte an der Kathode zur Bewirkung einer elektrolytischen Aufbringung der Übergangsmetall-Legierungselemente in amorpher Form auf das Substrat; und c) Aufbringen einer Beschichtung von Gold mit einer Dicke zwischen 0,0254-0,762 µm (1 bis 30 microinches) auf die elektrolytisch aufgebrachte amorphe Übergangsmetallegierung, um eine elektrische Kontaktstruktur mit unbedeckter Goldoberfläche zu schaffen.

6. Verfahren nach Anspruch 5, dadurch gekennzeichnet, daß der Schritt a) durchgeführt wird, indem man ein Plattierungsbad verwendet, das Phosphorsäure und Nickel allein, oder Nickel und Kobalt enthält.

7. Verfahren nach Anspruch 5, dadurch gekennzeichnet, daß der Schritt b) so durchgeführt wird, daß die Temperatur des Bades zwischen etwa 70-85°C liegt und daß die Stromdichte an der Kathode zwischen etwa 1076,49687,6 Amp/m² (100-900 amp/ft²) beträgt und eine elektrolytische' Aufbringung des amorphen Materials derart bewirkt wird, daß es eine Dicke von etwa 0,635-25,4 pm (25-100 microinches) hat; und daß der Schritt a) durchgeführt wird, indem in das Plattierungsbad zwischen 0,1 Mol/It und der Löslichkeitsgrenze lonen zugesetzt werden, die aus der Gruppe bestehend aus lonen von TiFₑ- SiFₛ- und ZrFₛ- ausgewählt sind.

8. Verfahren nach Anspruch 7, dadurch gekennzeichnet, daß die Schritte a) und b) derart ausgeführt werden, daß die amorphe Legierung, die auf das Substrat aufgebracht wird, eine Nickel-Kobalt-Phosphorlegierung ist, die etwa 15-25 Atomprozent Phosphor und mindestens 5 Atomprozent Kobalt aufweist.

9. Verfahren nach Anspruch 5, dadurch gekennzeichnet, daß der Schritt c) durchgeführt wird, um eine Beschichtung aus hartem Gold mit einer Dicke zwischen 0,127-0,381 um (5-15 microinches) aufzubringen.

## Revendications

1. Contact électrique ayant une résistance de contact, aussitôt après sa fabrication, qui est inférieure à 4 milliohms, comprenant un substrat conducteur électriquement, un alliage d'un métal de transition amorphe déposé sur ce substrat et un placage non recouvert d'or par dessus l'alliage de métal de transition amorphe, ce placage d'or ayant une épaisseur comprise entre environ 0,0254 et 0,762 micromètre.

2. Contact électrique suivant la revendication 1 caractérisé en ce que 1 alliage de métal de transition amorphe est un alliage du type nickel phosphore.

3. Contact électrique suivant la revendication 2 caractérisé en ce que l'alliage nickel-phosphore a une teneur d'environ 15 à 25% atomique de phosphore et une teneur d'environ 5 à 15% atomique de cobalt.

4. Contact électrique suivant la revendication 3 caractérisé en ce que le placage d'or non recouvert est de l'or dur ayant une épaisseur comprise entre environ 0,127 micromètre et 0,381 micromètre.

5. Procédé de fabrication d'un contact électrique caractérisé en ce qu'il comprend les étapes consistant à; a) immerger un substrat conducteur électriquement dans un bain de placage comportant des éléments d'alliage d'un métal de transition; b) contrôler les conditions de température du bain et la densité du courant à la cathode afin d'effectuer un dépôt électrolytique das éléments d'alliages de métal de transition, sous forme amorphe, sur le substrat; et c) appliquer un placage d'or ayant une épaisseur comprise entre 0,0254 et 0,762 micromètre sur l'alliage de métal de transition amorphe déposé électrolytiquement afin de produire une structure de contact électrique ayant une surface d'or non recouverte.

6. Procédé suivant la revendication 5 caractérisé en ce que l'étape a) est réalisée en utilisant un bain de placage contenant de l'acide phosphorique et du nickel seul ou bien du nickel et du cobalt.

7. Procédé suivant la revendication 5 caractérisé en ce que l'étape b) est réalisée de telle façon que la température du bain soit comprise environ 70-85°C et que la densité de courant à la cathode soit comprise entre environ 1076,4-9687,6 Alm² et de manière à effectuer un dépot électrolytique du matériau amorphe tel qu'il ait une épaisseur d'environ 0,635-25,4 micromètres; et en ce que l'étape (a) est réalisée en incorporant dans le bain de placage entre 0,1 molaire et à la limite de solubilité d'ions choisis dans le groupe constitué par les ions TiFs-, SiFₛ- et ZrFₛ-.

8. Procédé suivant la revendication 7 caractérisé en ce que les étapes a) et b) sont réalisées de telle façon que l'alliage amorphe déposé sur le substrat-soit un alliage du type nickel-cobalt-phosphore, ayant une teneur d'environ 15-25% atomique de phosphore et une teneur d'au moins 5% atomique de cobalt.

9. Procédé suivant la revendication 5 caractérisé en ce que l'étape c) est réalisée de manière à appliquer un placage d'or dur ayant une épaisseur comprise entre 0,127-0,381 micromètre.
